

# United States Patent Office

**3,023,092**

Patented Feb. 27, 1962

1

**3,023,092  
MOTOR FUEL**

Edwin O. Hook, Chagrin Falls, and David P. Tate, Northfield, Ohio, assignors to The Standard Oil Company, Cleveland, Ohio, a corporation of Ohio  
No Drawing. Filed June 4, 1950. Ser. No. 818,007

No Drawing. Filed June 4, 1959, Ser. No. 818,007  
1 Claim. (Cl. 44-69)

This invention relates to an improved motor fuel composition and in particular to a leaded fuel composition for high compression, spark-ignition engines containing an organic phosphorus compound.

It is a well-recognized fact today that during the operation of an initially clean internal combustion engine on gasoline-type fuels deposits form progressively and accumulate on the walls of the combustion chamber and on the terminals of sparkplugs. These deposits cause plug fouling, raise octane number requirement of the engine, and in general reduce appreciably the efficiency of the engine. The deposit problem is particularly aggravated when tetraethyl lead is contained in the fuel since the deposits now have a metallic nature which manifests a more harmful effect on engine operation than deposits which are essentially of carbonaceous character. In order to obtain a high octane number fuel such as is required for modern high compression internal combustion engines, most fuels require the addition of tetraethyl lead and hence the deposit problem in the combustion zone becomes aggravated.

A number of compounds of phosphorus have been proposed in the past for addition to gasoline to alleviate these adverse effects of deposits and particularly lead deposits which form in the combustion zone of the engine. One of the chief objections to the use of such phosphorus compounds, however, is that they characteristically lower to some extent the octane number of the fuel which obviously negates in part the advantage gained in the first instance when tetraethyl lead is added to the fuel.

In accordance with the present invention, it has been found that the addition of diethyl N-(2,4-dimethyl phenyl) amido phosphite to a gasoline in amounts to supply the quantity of elemental phosphorus normally required to alleviate the adverse effects on deposit problems quite surprisingly increases the octane number of the fuel.

The diethyl N-(2,4-dimethyl phenyl) amido phosphite compound for use in the fuel of the invention is a known chemical and may be prepared by reacting diethyl chlorophosphite with 2,4-dimethyl aniline in benzene.

The reaction proceeds according to the following equation:



The amount of diethyl N-(2,4-dimethyl phenyl) amido phosphite to be incorporated in the fuel of the invention depends to some extent upon the particular fuel employed as well as the amount of tetraethyl lead which is included therein. Amounts of the compound from 0.004% to 0.08% by weight based on the total fuel may be used effectively.

It is intended that the motor fuel of the invention may also include other known additives for commercial fuels, such as oxidation inhibitors, gum inhibitors, dyes, solvent oils, and the like.

2

When tetraethyl lead is used, the fuel may also contain a lead scavenging agent such as a volatile alkyl halide or a mixture of volatile alkyl halides such as ethylene dichloride and/or ethylene dibromide. These halides are usually present as 1 theory of ethylene dichloride and  $\frac{1}{2}$  theory of ethylene dibromide (the so-called "motor mix") or 1 theory of ethylene dibromide (the so-called "aviation mix"). By "theory" is meant the stoichiometric amount of the ethylene dihalide for combination with all of the lead as lead halide.

10 The base gasoline for the fuel can comprise a mixture of hydrocarbons boiling in the gasoline range and can be either a straight-run gasoline or a gasoline obtained from a conventional cracking process, or mixtures thereof.

15 The base gasoline may also contain components obtained from various other refinery processes, such as alkylation, isomerization, hydrogenation, polymerization, catalytic reforming, or combinations of two or more of such processes.

20 To demonstrate the beneficial octane effect obtainable when operating an engine with the fuel of the invention, octane ratings were made in an ASTM single-cylinder engine in accordance with a test procedure referred to as the Research Method. The operating conditions for this 25 ASTM engine, when running the Research Method determination, is set forth in ASTM D908-55. A device is installed in the cylinder head of this ASTM engine so that the pressure impulses from detonation can be detected. These are electronically amplified and their intensity indicated on a knock meter on the engine panel board. The motor fuels to be tested are used as the fuel for the engine. The test fuels are compared in knock intensity with that of various reference fuels which are blends of two standard compounds—iso-octane (2,2,4-trimethyl pentane) which is assigned an arbitrary number of 100 for the test, and n-heptane which is assigned an arbitrary number of 0. A blend of iso-octane and n-heptane is found which produces the same knock intensity as the fuel under test. The percentage by volume of iso-octane and the matching blend is designated as the octane number of the gasoline. For example, if a blend of 80% iso-octane and 20% n-heptane is required to duplicate the knock intensity of the test fuel, the fuel would then be given an octane number of 80. The base gasoline was 40 the same for all the fuels tested. Fuel 1 contained 0.016% by weight diethyl N-(2,4-dimethyl phenyl) amido phosphite in accordance with the invention. For comparison, fuels 2 and 3 contained phosphorus compounds which have previously been proposed as gasoline additives 45 and which are now in commercial usage. The base fuel had the following compositions and specifications:

**Composition, vol. percent:**

|      |                           |      |
|------|---------------------------|------|
| 1 55 | Saturates                 | 49.7 |
|      | Olefins                   | 10.3 |
|      | Aromatics                 | 40.0 |
|      | Tetraethyl lead, cc./gal. | 2.0  |
|      | Reid vapor pressure       | 11.5 |

### ASTM distillation, ° F.:

| ASTM distillation, °F. |       | 91<br>121<br>173<br>231<br>272<br>320<br>390 |
|------------------------|-------|----------------------------------------------|
| 60                     | I.B.P |                                              |
|                        | 10%   | -----                                        |
|                        | 30%   | -----                                        |
|                        | 50%   | -----                                        |
|                        | 70%   | -----                                        |
| 65                     | 90%   | -----                                        |
|                        | E.P.  |                                              |

The results of the test are found in the table below:

| Fuel      | Additive                                         | Concen-<br>tration,<br>percent<br>by<br>weight,<br>phos-<br>phorous | Octane<br>rating | Change<br>in octane<br>rating<br>over base<br>fuel |
|-----------|--------------------------------------------------|---------------------------------------------------------------------|------------------|----------------------------------------------------|
| Base fuel | None                                             | None                                                                | 100.4            |                                                    |
| 1.....    | Diethyl N-(2,4-dimethyl phenyl) amido phosphite. | 0.0021                                                              | 100.7            | +0.3                                               |
| 2.....    | Tricresyl phosphate.....                         | 0.0021                                                              | 100.1            | -0.3                                               |
| 3.....    | Dimethyl xylol phosphate.....                    | 0.0021                                                              | 100.2            | -0.2                                               |

As will be noted from the above table, the addition of diethyl N-(2,4-dimethyl phenyl) amido phosphite to the base fuel produced a definite positive effect on octane number. By contrast, it is obvious that known phosphate esters added to the fuel for the same test demonstrate a definite negative effect upon octane number.

The invention has been described hereinabove with reference to various specific examples and embodiments.

It will be understood that the invention is not limited to such examples and embodiments but is intended to have such scope as afforded by the appended claim.

We claim:

5 A leaded gasoline fuel containing an octane increasing phosphorus additive consisting of from 0.004% to 0.08% by weight diethyl N-(2,4-dimethyl phenyl) amido phosphite.

References Cited in the file of this patent

UNITED STATES PATENTS

|           |                   |               |
|-----------|-------------------|---------------|
| 2,617,794 | Anderson          | Nov. 11, 1952 |
| 2,878,255 | Toy et al.        | Mar. 17, 1959 |
| 2,892,691 | Howell            | June 30, 1959 |
| 2,897,068 | Pellegrini et al. | July 28, 1959 |
| 2,911,431 | Orloff et al.     | Nov. 3, 1959  |

FOREIGN PATENTS

|         |           |               |
|---------|-----------|---------------|
| 216,009 | Australia | July 11, 1958 |
| 565,182 | Canada    | Oct. 28, 1959 |